

M. Nelson,

Casting Soft Metal Articles.

N<sup>o</sup> 17,109.

Patented Apr 21, 1857.

Fig. 1



Fig. 2



Fig. 3.



# UNITED STATES PATENT OFFICE.

MORTIMER NELSON, OF NEW YORK, N. Y.

## IMPROVEMENT IN MOLDS FOR CASTING.

Specification forming part of Letters Patent No. **17,109**, dated April 21, 1857.

*To all whom it may concern:*

Be it known that I, MORTIMER NELSON, of the city, county, and State of New York, have invented certain improvements in the manufacture of molds for casting britannia and other metals fusible below a red heat, of which the following is a full, clear, and exact description, reference being had to the accompanying drawings, making part of this specification, in which—

Figures 1 and 2 are interior views of the two halves of a mold prepared for casting one face of a medal; Fig. 3, a section through the same on the line A A.

Difficulty has been experienced in reproducing in metal, by casting, articles having highly-polished surfaces or fine lines—such as engraving or chasing—as the metallic mold, if made of sufficient thickness to obtain the desired strength, would chill the more fusible metal being cast in it before the delicate lines or parts had been filled; or if the mold were heated to prevent this the casting would be frosted or often filled with minute holes.

To obviate these objections and to obtain a mold that shall possess sufficient strength and rigidity without containing a mass of metal sufficient to chill the fluid metal being cast is the object of my present invention, which I will now proceed to describe, that others skilled in the art may understand the manner in which I have carried it out.

The said drawings represent a mold taken by my improved process from one side of a medal in the following manner: One half of the article to be molded is coated with black-lead in the usual way, and a thin sheet of copper is deposited on it by the electrolyte process. The other half is then treated in the same way, thus forming a perfect mold, even to the finest engraved lines of the articles. These thin sheets B, Fig. 3, are then backed up with plaster-of-paris to the requisite thickness, as at C, Fig. 3. The copper on its outer surface, being rough, as deposited in the bath, serves to hold

the plaster to it and prevent the sheet of copper from springing or warping when the hot metal is poured into it. This backing C is then coated with black-lead and the whole mold is placed in a copper bath, and the sheet of copper D is deposited on the rear and ends of the backings, the interior of the mold being protected from the deposit in the usual manner. If the article to be molded is of such a form as to require the mold to be made of more than two pieces, each portion of it is formed as above described.

By the above process I obtain a mold having all the advantages of one of solid metal without the disadvantage of chilling the fluid metal when poured into it, enabling me to reproduce, in any metal fusing at a less heat than copper, castings having fine engraved lines or devices in a better manner and at a much less cost than has been heretofore practicable.

When the metal employed for casting fuses at a temperature more nearly approaching that of the mold it is liable to adhere to the copper. To prevent this the face of the mold may be brushed over with a thin coating of black-lead; or it may be smoked before pouring in the hot metal. For the same purpose the face of the mold may be plated by the electrolyte process with a thin coat of iron, to which the fused metal will not adhere, and which tends to render the mold more durable than when the casting is made upon a surface of copper.

What I claim as my invention, and desire to secure by Letters Patent, is—

The within-described method of forming molds for casting britannia and other metals by backing up a thin metallic face with plaster, in the manner substantially as herein set forth.

M. NELSON.

Witnesses:

WM. DIXEY,  
EDWARD BURKE.